

# UNITED STATES PATENT OFFICE.

FRANCIS J. HOBSON, OF GUANAJUATO, MEXICO.

## PROCESS OF SILVER EXTRACTION.

No. 828,288.

Specification of Letters Patent.

Patented Aug. 7, 1906.

Original application filed July 18, 1905, Serial No. 270,300. Divided and this application filed December 20, 1905. Serial No. 292,556.

To all whom it may concern:

Be it known that I, FRANCIS J. HOBSON, a citizen of the United States, now residing at Guanajuato, in the Republic of Mexico, have 5 invented certain new and useful Improvements in Processes of Silver Extraction, of which the following is a specification.

My present invention consists of an improved process for extracting silver from its 10 ores, and particularly from ores in which the silver is present in combination with sulfur. Sulfur being present in almost all silver ores, the improved process is of very general application.

15 Briefly outlined, the process consists of treating the ores after such preliminary sizing as may be desired with a solution containing a mercurous potassic cyanid. This salt, the characteristics of which are described in my previous application, Serial No. 270,300, filed July 18, 1905, of which the present case is a division, has a selective affinity for silver in combination with sulfur. This selective affinity I have demonstrated 20 experimentally a great many times. The formula of the salt is  $\text{KHgCy}_2$ . It forms with silver, when in combination with sulfur, a double salt—the cyanid of silver and potassium—which is freely soluble in water, and 25 also the sulfid of mercury, which is substantially insoluble in water and passes off with the tailings. The reaction to which I here refer is expressed verbally as follows: Silver sulfid plus mercurous potassic cyanid equals 30 cyanid of silver and potassium plus sulfid of mercury, and in chemical symbols the reaction is expressed thus:



40 The solvent which I employ in my improved process does not attack gold in any of the forms in which it appears to exist in ore, and although it forms the same salt of silver and potassium in solution as cyanid of potassium when the latter dissolves silver it does not do so in the same way, since potassium cyanid dissolves silver by the well-known Elsner's equation, stated verbally as follows: Silver plus cyanid of potassium plus oxygen 45 plus water equals cyanid of potassium and silver plus potassium hydrate or caustic potash. This equation in chemical symbols is stated thus:



The same equation applies to the solution of gold, gold replacing silver in it.

Free oxygen in solution is necessary to dissolve silver or gold and form the double salt of potassium and silver or gold with cyanogen. 60

I may produce the mercurous potassic cyanid in any desired way, since the particular method of its production does not seem to affect the results. I may, for example, add mercurous chlorid ( $\text{Hg}_2\text{Cl}_2$ ) to a solution of 65 potassium cyanid, ( $\text{KCy}$ .)

Another method which I may use is to add mercuric chlorid (corrosive sublimate,  $\text{HgCl}_2$ ) to the ordinary mill cyanid solutions containing ferrocyanid of potassium, in which case 70 the reaction may be stated verbally thus: Ferrocyanid of potassium plus mercuric chlorid equals ferrocyanid of mercury plus chlorid of potassium. This reaction may be expressed in chemical symbols as follows: 75



This is succeeded by the following reaction: Ferrocyanid of mercury plus cyanid of potassium equals ferrocyanid of mercury and potassium plus mercurous potassic cyanid. 80 This reaction may be expressed in chemical symbols as follows:



The most suitable strength of the solution is to some extent dependent upon the silver content of the ore and the form in which the metal is present. I have obtained good results with solutions varying from .05 to .50 per cent. The metal may be separated from the solution in any of the approved methods commonly employed in cyanid processes, such as precipitation by zinc dust or shavings or electrolysis. 95

The solution should be kept alkaline, and this may be effected by the addition of any suitable alkali, such as caustic potash or soda, although in most cases lime will be 100 found to be not only the cheapest, but the best alkali. This application is restricted to that form of my invention in which the mercurous potassic cyanid is formed by the addition of mercuric chlorid to a solution containing ferrocyanid. The other methods of obtaining the solvent, mercurous potassic cyanid, are intended to be broadly covered by my application Serial No. 292,554, filed December 20, 1905, which is a division of the 110

parent case, Serial No. 270,300, hereinbefore referred to.

Having thus described my invention, what I claim, and wish to protect by Letters Patent of the United States, is—

1. The process of extracting silver from its ores, which consists of subjecting the ores to the action of a solution of cyanid and ferrocyanid of an alkaline metal, to which has been added mercuric chlorid.

2. The process of extracting silver from its ores, which consists of subjecting the ores to the action of a solution of ferrocyanid of potassium to which has been added mercuric chlorid.

3. The process of extracting silver from its ores, which consists in subjecting the ores to

the action of a solution of the cyanid of an alkaline metal to which has been added ferrocyanid of potash and mercuric chlorid.

4. The process of extracting silver from its ores, which consists of adding to a mill solution containing cyanid and ferrocyanid of potash, a mercuric chlorid.

5. The process of extracting silver from its ores, which consists of subjecting the ores to the action of a solution of cyanid and ferrocyanid of potash in the presence of a chlorid of mercury and an alkali, and subsequently precipitating the silver from the solution.

FRANCIS J. HOBSON.

Witnesses:

W.M. C. YOUNG,  
H. D. CLEEDER.